

## UNITED STATES PATENT OFFICE.

ROBERT STEWART CARMICHAEL, JAMES CARMICHAEL, AND FREDERIC ROBERT CARMICHAEL, OF PARIS, FRANCE.

## PROCESS OF OILING AND FINISHING TEXTILE MATERIALS.

SPECIFICATION forming part of Letters Patent No. 761,203, dated May 31, 1904.

Application filed August 27, 1902. Serial No. 121,203. (No specimens.)

*To all whom it may concern:*

Be it known that we, ROBERT STEWART CARMICHAEL, JAMES CARMICHAEL, and FREDERIC ROBERT CARMICHAEL, citizens of the French Republic, residing at 15 Rue du Louvre, Paris, France, have invented new and useful Improvements in Processes of Oiling and Finishing Textile Materials, of which the following is a specification.

10 Finishes the basis of which is starch, amy-  
lum, or dextrines have all the drawbacks of  
imperfectly maintaining the filling substances  
or dressings which they are intended to fix  
either on raw textile materials or on yarn or  
15 fabrics, so that the advantage that it is in-  
tended to obtain by the loading of the textile  
materials with such substances is only illusory,  
because this incompletely-fixed loading falls  
out as dust during the mechanical operations  
20 of working the textile materials, (carding,  
combing, spinning, and weaving.)

It has not hitherto been possible to effect in  
a single process the operations of oiling and  
loading and finishing textile materials so as  
25 to preserve the loading fixed during the opera-  
tions hereinbefore mentioned.

Our improved process has for its object,  
first, to effect the oiling, finishing, (sizing,) and loading by the use of a single bath hav-  
30 ing a casein base, the operation being carried  
out either by steeping or by means of a me-  
chanical oiler; secondly, to finish (size) and  
load the tissues, yarn, or raw textiles in a du-  
rable manner by the use of casein as the means  
35 for fixing the loading or inert substances.

Our process is based on the colloidal prop-  
erty of casein, its plasticity, and the faculty it  
possesses of forming with mineral oils soapy  
40 solutions which are caseinic and capable of  
being mixed with one another and also of hold-  
ing in suspension a very large proportion of  
inert or heavy substances.

The proportion of the substances compos-  
ing the bath employed for the carrying out of  
45 our process may vary according to the nature  
of the materials to be treated. Thus in the  
case of raw textiles the proportion of min-  
eral oil or fatty material added is about six  
times as much as that of the casein, while when

treating spun or woven textiles the fatty ma-  
terial added is much weaker than that of the  
casein—say about six times less than the lat-  
ter. In a general way the baths that we pre-  
fer to employ have, according to circum-  
stances, one of the two following composi- 55  
tions:

First. In case we wish to treat a raw textile  
material in view of its oiling, finishing, load-  
ing the bath has the following composition:  
casein, sixteen parts; soap, eight parts; car-  
bonate of soda or other alkaline substances,  
two parts; mineral or like oil, sixty parts;  
water, three hundred parts; loading sub-  
stances, two hundred parts. This bath is pre-  
pared in the following manner: Powdered car-  
bonate of soda is mixed with casein, which is  
also in powder, and the mixture is put to steep  
for an hour in a cold soapy solution, and then  
the oil is incorporated and the whole is heat-  
ed in a water-bath, agitating it, but not allow-  
ing it to boil. The inert substances are then  
mixed with this solution and the whole is  
passed through a sieve. This solution, main-  
tained at a heat of about fifty degrees, is ap-  
plied to the raw or scoured textile materials 75  
by means of an oiler in the ordinary manner  
as if the oiling alone were being effected. At  
least three hundred liters of the bath herein-  
before specified must be employed per eight-  
een hundred kilograms of material. The tex-  
tile material thus oiled, loaded, and finished  
then undergoes the ordinary operations of  
spinning, weaving, and the like. 80

Secondly. For loading and finishing warp or  
fabric the operation is preferably carried out 85  
at the moment of sizing or by immersing the  
hanks. For preparing the bath of loading  
finish there is employed casein, twelve parts;  
mineral oil, two parts; soap, four parts; kao-  
lin, seventy parts; water, two hundred parts; 90  
dry carbonate of soda, 1,500 parts, and we op-  
erate with this bath in the same way as for the  
ordinary sizing.

It is quite evident that the quantities herein-  
before mentioned will vary with the loading, 95  
flexibility, and finish to be obtained, knowing  
that per kilogram of inert substances to be  
fixed sixty grains of dry casein must be used.

Instead of dry casein hydrated casein might be employed—such, for instance, as soft skim-milk cheese—taking into account the water of hydration.

5 Having now particularly described and ascertained the nature of the said invention and in what manner the same is to be performed, we declare that what we claim is—

10 The process permitting to simultaneously effect the oiling, finishing and loading of raw textile materials, and the treatment of spun or woven textiles, consisting in submitting these materials to the action of a particular bath prepared by diluting casein, its mineral

acidity being neutralized by the addition of 15 just sufficient carbonate of soda, in a watery solution of soap, and by adding to this bath the fatty materials necessary for the finishing, and the material used for loading.

In witness whereof we have hereunto set 20 our hands in the presence of two witnesses.

ROBERT STEWART CARMICHAEL.  
JAMES CARMICHAEL.  
FREDERIC ROBERT CARMICHAEL.

Witnesses:

EDWARD P. MACLEAN,  
JULES FAYOLLET.